

July 5, 1960

A. WACHTER ET AL

2,943,909

CORROSION- AND FUNGUS-INHIBITING COMPOSITION

Filed Aug. 26, 1957

- A SODIUM NITROPHENATE
- B AMINE PHENATE
- C AMINE PHENATE + AMINE NITRITE
- D SODIUM PHENATE + AMINE NITRITE



FIG. 1



FIG. 2

INVENTORS:  
AARON WACHTER  
RITA WIELAND  
BY: *William H. Myers*  
THEIR AGENT

1

2,943,909

## CORROSION- AND FUNGUS-INHIBITING COMPOSITION

Aaron Wachter, Oakland, and Rita Wieland, Berkeley, Calif., assignors to Shell Oil Company, a corporation of Delaware

Filed Aug. 26, 1957, Ser. No. 680,162

6 Claims. (Cl. 21—2.7)

This invention is concerned with compositions useful for the reduction in fungus growth and corrosion. More particularly, it is directed to compositions useful for the prevention of corrosion of metallic surfaces and simultaneous inhibition of fungus growth during storage of metals.

One of the most pressing problems in the storage of metallic items is corrosion of their surfaces due to the presence of oxygen and water vapor. Corrosion can be inhibited by smearing the metallic parts with an oil or grease-like material or by coating them with a strip plastic composition. However, each of these involve manual operations adding to the cost of preparation of storage and elimination of the protective coating before the article can be used. A much more convenient and less costly means of inhibiting corrosion comprises confinement of the metallic parts in an enclosed space such as by paper or other wrapper and including in the enclosed space a corrosion inhibitor chosen to volatilize slowly but effectively during the storage period, thus providing a constant means of protecting the surface against corrosion without necessitating the manual preparation or cleaning of the article for this purpose. Such inhibitors are normally referred to as "vapor phase inhibitors." The most effective class of such items comprises the amine nitrites and certain mixtures of these preferably containing a basic acting agent so as to maintain a pH at least above about 6.0.

Under certain conditions such as high humidity and/or high temperature, one complicating factor appears in the use of vapor phase inhibitors, namely, the growth of fungus within the enclosed space and consequent interference with the process of vapor phase corrosion inhibition. While it is true that fungus growth normally occurs on organic surfaces such as cloth or plant fibers or the like, under many tropical conditions it has been found that fungi grow on other surfaces as well, such as glass, metal, wood, etc. Under these conditions and particularly when the fungus grows or touches the metal surface it has been found that vapor phase corrosion inhibition of that area so effected is not satisfactory and rusting or corrosion occurs.

It is an object of the present invention to provide a means for controlling both corrosion and fungus growth. It is another object of this invention to provide an improved vapor phase inhibiting composition which is also fungicidal. It is a further object of this invention to provide a means of preventing corrosion and simultaneous fungus growth inhibition. It is a further object to provide a wrapping material having these properties. Other objects will become apparent during the following description of the invention.

Now, in accordance with the present invention, it has been found that vapor phase corrosion inhibiting compositions also having fungicidal properties comprise 10—90% by weight of a water soluble nitrite salt and 90—10% by weight of an organic nitrogen base salt of a phenol, said phenol having a molecular weight less than about

2

350, both salts having vapor pressures of at least about 0.00002 to mm. Hg at 21° C. Still in accordance with the present invention wrapping materials are provided comprising a solid inactive packaging material, such as 5 paper, having the above compositions physically associated therewith. Also according to the invention a method is provided for inhibiting fungicidal growth (on organic or inorganic surfaces) and corrosion by maintaining a metal in the immediate presence of an atmosphere containing the two salts as stated above.

Free phenols cannot be mixed with nitrite salt since, due to the acidic nature of the phenol, the nitrite salts are rapidly decomposed. It is possible to combine a metallic salt of a phenol with a nitrite salt but for some reason this has been found to drastically reduce the rate of vaporization of the nitrite salt. Since it is highly desirable to maintain the original rate of vaporization of the nitrite salt so that efficient and complete corrosion inhibition is maintained, it therefore is undesirable to combine 20 metallic salts such as sodium phenates with the nitrite salt.

It has been found, however, that the amine salts of phenols do not adversely affect the rate of vaporization of the nitrite salt. Conversely, the presence of nitrite 25 salts has been found to cause rapid depletion of the concentration of sodium salts of phenols from their compositions, either by increasing the rate of vaporization or by actual decomposition of the metallic salt of the phenol. On the other hand, however, the combination of nitrite 30 salts with amine salts of phenols causes substantially no change in the rate of vaporization of the amine phenate than that experienced when the latter is utilized in the absence of the nitrite salt. Consequently, it will be seen that the present invention takes advantage of these 35 two sets of phenomena in utilizing the combination of the amine phenate and the amine nitrite for the combined purpose of corrosion inhibition and fungicidal properties without adversely affecting the rates of vaporization of either the nitrite or the phenate. Furthermore, 40 it has been found that a moderate synergistic effect is experienced with respect to corrosion inhibition by the combination of the two materials.

The nitrite salts can be utilized as inorganic salts either metallic or ammonium but preferably are organic 45 base salts and more particularly, the organic nitrogen base nitrites. The nitrites and the phenates can be prepared from the same classes of organic bases, particularly organic nitrogen bases, or may be utilized in the form of different organic base salts.

50 Representative classes of organic bases which are suitable for preparing the salts used as vapor phase inhibitors according to the present invention include: primary amines, secondary amines, tertiary amines, cyclic secondary amines of the type of piperidine, oxazines, morpholine, thiazolines, and pyrrolidines; and various nitrogenous bases such as urea, thiourea, hydrazines, hydroxylamines, amidines, and guanidine. In any of the above nuclei, alkyl cycloalkyl, terpinyl, bornyl, aralkyl, benzyl, phenyl, aryl and various substituent groups or atomic 55 radicals may be present so long as the sum total basicity of the nitrogenous compound is approximately equal to or greater than the acidity of nitrous acid with which it forms a salt. Among the substituent groups the alkyl and cycloalkyl groups are preferred.

60 The basicity of the various basic constituents of the class of salts disclosed herein is described, for example, in "The Organic Chemistry of Nitrogen," by N. V. Sidgwick, 1937 edition, and in "Organic Chemistry," by Paul Karrer, 1938 edition.

65 More specifically and preferably, organic nitrogen base salts of nitrous acid include the following nitrite salts of: (1) Primary amines, such as (a) primary amines in

which the amine group is attached to a secondary or a tertiary aliphatic carbon atom as in the following structural formulas:



5

wherein R<sub>1</sub>, R<sub>2</sub> and R<sub>5</sub> are hydrocarbon radicals which are aliphatic, alicyclic, heterocyclic, aromatic, or alkylated cyclic radicals, and may, if desired, contain preferably not more than one olefinic double bond, or R<sub>1</sub> and R<sub>2</sub> are joined in the form of a cyclo-aliphatic or heterocyclic-aliphatic ring radical R<sub>5</sub>; (b) primary amines in which the amine group is attached to an aralkyl group as in the following structural formula:



wherein R<sub>4</sub> is an aromatic hydrocarbon radical, preferably a phenyl or alkylated phenyl radical and n is an integer which is preferably 1 or 2; (c) primary aliphatic amines, such as methyl amine, which react with nitrous acid in the presence of an excess of the amine to give a primary amine nitrite salt (as distinguished from a primary aliphatic amine which reacts with nitrous acid to yield nitrogen, an alcohol, or other reaction products).

(2) Secondary amines, such as those in which the amine group is attached to an aliphatic carbon atom, preferably a secondary or tertiary carbon atom, as represented by the following structural formulas:



10

wherein R<sub>1</sub> and R<sub>2</sub> are hydrocarbon radicals as in 1 (a) and wherein R<sub>1</sub> and R<sub>2</sub> may be joined in the form of a ring forming



15

which is either N-alicyclic or contains in the R<sub>3</sub> portion of the organic ring atoms of the type of oxygen and/or sulfur.

(3) Tertiary amines.

(4) Quaternary ammonium bases including pyridinium bases.

Specific examples of organic nitrogen bases suitable for preparation of the amine-nitrite salt vapor phase corrosion inhibitors of the present invention include:

Primary amines: methylamine, isopropyl amine, 2-amino-butane, tertiary butyl amine, 2-amino-4-methylpentane, various amyl, hexyl, heptyl, octyl, and higher homologous primary amines wherein the amine group is attached to a secondary or tertiary carbon atom; cyclopentyl amine, alkylated cyclopentyl amines, cyclohexylamine, monomethylcyclohexylamines, dimethyl cyclohexylamines, trimethyl cyclohexylamines, other alkylated cyclohexylamines, bornyl amine, fenchyl amine, cyclo-terpenyl amines, pinyl amine, benzylamine, betaphenyl-ethylamine, alkylated benzylamines, tetrahydro betanaph-thylamine, allyl amine, beta-methyl allyl amine, beta-chloro allyl amine, and their homologs and analogs.

Secondary amines: di-methyl-, di-ethyl-, di-n-propyl-, di-isopropyl-, di-butyl-amines; various secondary amines derived from amyl, hexyl, heptyl, octyl, and higher homologous alkyl groups; methyl isobutyl amine, N-methyl N-tertiary-butyl amine, N-alkyl N-cyclohexyl amine, N-alkyl N-bornyl amine, di-bornyl amine, N-methyl N-cyclo-terpenyl amine, N-isopropyl N-(1)menthyl amine, N-alkyl N-benzyl amines and their homologs and analogs; dicyclopentyl amine, dicyclohexyl amine, alkylated di-cyclohexyl amines; diphenylamine, dibenzylamine, di(beta phenyl ethyl) amine; piperidine, piperazine, alkylated piperidines or piperazines; 1,4 - alkylated and un-alkylated oxazines such as morpholine and 2,4,4,6-tetra-

methyl tetrahydro-1,3-oxazine; alkylated-1,3-thiazolines such as 2,4,4,6-tetramethyl tetrahydro-3-thiazoline.

Secondary amine type derivatives of alkylene diamines, such as:



wherein R<sub>1</sub> and R<sub>3</sub> may be like or different aliphatic, alicyclic aralkyl, alkarylalkyl, heterocyclic, terpenic radicals, and wherein R<sub>2</sub> is an alkylene radical. These R<sub>1</sub> and R<sub>3</sub> radicals for instance, may be isopropyl, butyl, cyclohexyl, benzyl, and/or bornyl radicals. The R<sub>2</sub> radical is preferably an ethylene or propylene radical.

Tertiary amines: trimethyl amine, triethylamine, tri-n-propylamine, tri-isopropylamine, tributylamine, higher homologous and isomeric trialkylamines, variously N-substituted tertiary amines having different organic radicals on the amino nitrogen atom, e.g., alkyl, alicyclic, bornyl, fenchyl, aralkyl, and like homologs and analogs; and tertiary amine type derivatives of alkylene diamines.

Quaternary ammonium bases: tetramethyl and higher tetraalkyl ammonium bases; trimethyl benzyl-, trimethyl cyclohexyl-, tributyl decyl ammonium bases; various quaternary N-substituted ammonium bases having various organic radicals (of the type described above) on the quaternary nitrogen atom; pyridinium and alkylated pyridinium or quinolinium quaternary ammonium bases having an alkyl, cycloalkyl, or aralkyl group on the quaternary nitrogen atom, including methyl, butyl, cyclohexyl, benzyl groups and like homologs or analogs.

The various hydrocarbon radicals or groups of the above amines may also contain stable and inert polar substituent atoms or radicals, such as, chlorine, ether, thio-ether, alcohol, free amino, or nitro groups. Neutral ketone, ester and nitrile groups, and aliphatic unsaturation may also be present, particularly in the case of allyl and chlorallyl groups.

The phenols which may be combined with the above types of amines to form the amine phenates suitable for use in the present invention include any phenols and substituted phenols having molecular weight less than about 350. These include especially the nitro and chloro phenols although polyhydroxy phenols and alkyl phenols as well as phenol itself are useful for the preparation of fungicidal amine salts compatible with the nitrites forming the other essential components of the present compositions. Nitro phenols are the preferred derivative class useful for the preparation of amine salts. Examples of nitro phenols which are suitable for this purpose are ortho, meta and para-nitro phenol, 2,4- and 2,6-di-nitro phenol; 2-nitro-4,6-dimethyl phenol; 2-methyl-4-tertiary amyl-6-nitro phenol; 2,6-dinitro-4-isooctyl phenol; 4-nitro resorcinol-1,3; 3-nitro-4-hydroxy-benzyl alcohol; alpha-nitro-beta naphthol, etc.

Suitable amine salts of phenols are the following:

- 55 Dicyclohexylamine salt of 2,4-dinitrophenol  
Diisopropylamine salt of dinitrophenol  
Dicyclohexylamine salt of dinitro-o-cyclohexylphenol  
Diisopropylamine salt of dinitro-o-cyclohexylphenol  
Dicyclohexylamine salt of o-nitrophenol  
60 Diisopropylamine salt of o-nitrophenol  
Dicyclohexylamine salt of dinitro-o-cresol  
Dimethylamine salt of 4,6-dinitro-2-sec.-butylphenol  
Di-sec.-butylamine salt of 2,4-dinitro-alpha-naphthol  
Isopropylcyclohexylamine salt of 4-n-propyl-2-aminopheno-  
65 nol  
Di(2-ethylhexyl)amine salt of a mixture of isomeric di-  
aminophenols  
Diethanolamine salt of 2,4,5-trichlorophenol  
Dicyclohexylamine salt of o-chlorophenol  
70 Dicyclopentylamine salt of meta-chlorophenol  
Di(2-ethylbutyl)amine salt of mixed monobromophenols  
Dicyclohexylamine salt of 2,4-dichlorophenol  
Diisopropylamine salt of 2,4,5-trichlorophenol  
Ethanolamine salt of 2,4,6-trichlorophenol  
75 Diisobutylamine salt of para-chloro-ortho-cresol

- Diisopropylamine salt of mixed chloroxylenols  
 Diisopropylamine salt of o-benzyl cresol  
 Dicyclohexylamine salt of o-benzyl cresol  
 Dicyclohexylamine salt of o-phenyl phenol  
 Diisopropylamine salt of o-phenyl phenol  
 Dicyclohexylamine salt of p-benzyl phenol  
 Dicyclohexylamine salt of hydroquinone  
 Diethylamine salt of n-heptyl resorcinol  
 Dihexylamine salt of mixed cresols

As stated hereinbefore, it is possible to utilize inorganic nitrites as well as amine nitrites in the present compositions. These include the alkali metal nitrites such as sodium, lithium, or potassium nitrites as well as the alkaline earth metal nitrites including calcium and magnesium nitrites. Ammonium nitrite may be used in addition to or in place of other nitrite salts.

It is preferred practice when utilizing an inorganic nitrite to include together therewith 0.05-20 parts by weight of a diamide for each part of the inorganic nitrite.

Amides, which have been successfully used, fall into the groups of mono-amides, diamides, and polyamides. By the term mono-amide is meant a compound having the general formula



where R is an aliphatic group having from 1 to 18 or 25 or more carbon atoms. These include such amides as acetamide, propionamide, and N-butyramide, N-valeramide, stearamide, palmitylamide, fatty acid amides, and the like. Although less activity results when R is aromatic or aliphatic-aromatic, amides of that type may be used. For example the amide component may be benzamide and the aromatic acid amides of the type benzene sulphonic acid amide, toluene sulphonic acid amide, naphthalene sulphonic acid amide, and the like.

Best use is made of the diamides having the formula



where R is hydrogen or an organic radical of the type previously described. Illustrative of suitable diamides are urea, N-substituted ureas, and unsymmetrical ureas, such as N-N-dibutyl urea, N-butyl urea, N-propyl urea, dimethyl urea, t-butyl urea, ti-amyl urea, and the like, and other diamides, such as buramines (the reaction product of amines such as butyl amine with urea), the reaction product of amines with biuret, and guanidine and derivatives thereof. A suitable polyamide is illustrated by biuret.

It is especially advantageous to ensure that the composition utilized has a pH above about 6.0. This can be effected by addition of such basic acting agents as are referred to in U.S. Patent 2,752,221.

The amine salts of the phenols may be prepared by simply dispersing the phenol and the amine in solvents, mixing them and thereafter evaporating the solvent. The same is true of the preparation of amine nitrites although it is preferred to form a solution of an amine phosphate and add thereto a solution of sodium nitrite or potassium nitrite in order to form the resultant amine nitrite. Methods of the latter type are disclosed in U.S. Patent 2,717,843. It is, of course, possible to utilize a combined process so that the mixture of nitrite and phenate may be formed in a single process rather than separately. Such a process comprises formation of a solution of an amine phosphate, preferably in alcohol or aqueous alcohol, followed by addition thereto of a solution (alcoholic) of the phenol in an amount sufficient to form an amine phenate with only a portion of the amine phosphate, the third step being the addition of sufficient nitrite such as sodium nitrite to react with the remaining portion of amine phosphate, thus creating a mixture of amine nitrite and amine phenate.

The vapor phase corrosion inhibitor and fungicide both

- should preferably have vapor pressures in excess of about 0.00002 mm. Hg at 21° C. and better results are obtained with a composition in which both of the nitrite and the phenate have vapor pressure greater than about 5 0.0001 mm. Hg at 21° C. The compositions are useful for preventing the corrosion and inhibiting fungus growth upon various ferrous metals such as steels and as well as combinations of steel with zinc or copper or other metals and aluminum as well as alloys of these metals.
- 10 Of course, the compositions also will inhibit or prevent fungus growth on other organic or inorganic surfaces (such as cloth, paper or other packaging materials) with which they come in contact.

- In one of the preferred embodiments of the present invention it is found advantageous to utilize a solid wrapping material such as paper which has been impregnated with the compositions disclosed herewith. The metal articles are then wrapped in the paper to obtain the dual inhibiting functions of the composition. On the other 15 hand, of course, it is possible to simply dispose the composition in powdered form or otherwise in metal articles such as cylinders or the like in order to prevent corrosion and inhibit fungus growth. While it is preferred under most circumstances to utilize compositions containing from 25 to 75% of either the nitrite or the phenate, it is also possible to utilize from 10-90% of the nitrite and 90-10% of the phenate dependent upon the severity of corrosion or of fungus growth as well as the humidity and temperature conditions involved in a specific use.
- 20 30 The following compositions illustrate the type of compositions useful for use in the present invention:

Composition A:

- 50% dicyclohexylamine nitrite  
 50% diisopropylamine-o-nitrophenate

Composition B:

- 25% diisopropylamine nitrite  
 75% diisopropylamine salt of 2,4-dinitrophenol

Composition C:

- 75% diisobutylamine nitrite  
 25% dicyclohexylamine salt of mixed cresols

Composition D:

- 30% sodium nitrite  
 30% urea  
 40% dicyclohexylamine salt of 2,4-dinitro-6-cyclohexylphenol

Composition E:

- 40% ammonium nitrite  
 30% N-butyl urea  
 30% ethanolamine salt of 2,4,6-trichlorophenol

Composition F:

- 85% diisopropylamine nitrite  
 15% diisopropylamine salt of 2,4,5-trichlorophenol

Composition G:

- 15% di-(2-ethylhexyl)amine nitrite  
 85% di(2-ethylhexyl)amine salt of 2,4-dinitro-o-cresol

*Example I*

- 60 When steel plates are wrapped in paper and stored under high humidity conditions at temperatures of about 90-110° F., rapid corrosion of the surface of the plate occurs. When storage is conducted while mold spores are present, it is found at the end of a one-month storage period that mold growth occurs on both the interior of the paper wrapper and on portions of the steel surface. When small amounts of dicyclohexylamine nitrite are present, the corrosion is reduced by a factor of 5 and when one-half of the nitrite is replaced with an equal 65 amount of dicyclohexylamine ortho nitrophenate, the corrosion rate was reduced by a factor of 75. At the same time, although mold spores are present and mold growth occurs when the phenate is not utilized, no mold growth is noted when the phenate is used for partial replacement 70 of the nitrite.

*Example II*

In order to determine the effect upon retention of phenates in contact with paper under conditions typical of those to be expected for storage of metallic parts, 60 pound kraft paper (A) was modified by depositing thereon 1.0 gram per square ft. of sodium ortho nitrophenate, on a second sample (B) the dicyclohexylamine salt of ortho nitro phenate, a third sample (C) containing a 50-50 mixture of the amine phenate and dicyclohexylamine nitrite and a fourth sample (D) containing sodium orthonitro phenate with an equal amount of dicyclohexylamine nitrite. These samples were exposed at room temperature (60-80° F.) in an active air stream and the amount of phenate remaining on the paper was periodically tested. Fig. I shows that the sodium or amine salts of the phenol when present alone on the paper had substantially the same rate of volatility or at least the same rate of retention on the paper. However, when these phenates were modified with an equal amount of the amine nitrite the rate of depletion of the sodium phenate increased sharply while the rate of depletion of the amine phenate remained substantially unchanged.

*Example III*

Samples C and D were analyzed periodically after exposure to the same conditions for amine nitrite retention. Also a sample E, containing 1 g./sq. ft. of the amine nitrite was tested under the same conditions. Fig. II shows that the addition of amine phenate to the amine nitrite did not substantially alter the rate of vaporization of the amine nitrite. However, the addition of sodium phenate resulted in a substantial reduction in the volatility of the nitrite.

We claim as our invention:

1. A composition comprising about 25-75% by weight of dicyclohexylammonium nitrite and about 75-25% by weight of dicyclohexylammonium nitrophenate.

2. A composition comprising about 25-75% by weight of a nitrite of the group consisting of dicyclohexylammonium nitrite and diisopropylammonium nitrite and about 75-25% by weight of a nitrophenate of the group consisting of cyclohexylammonium nitrophenate and di-cyclohexylammonium nitrophenate.

3. A substantially solid inactive packaging material having physically associated therewith a composition according to claim 1.

4. A substantially solid inactive packaging material having physically associated therewith a composition according to claim 2.

5. In a method for inhibiting both fungus growth on and corrosion of a metal normally corrodible by contact with water vapor and oxygen, the step comprising maintaining in the immediate presence of said metal an atmosphere containing a corrosion inhibiting and fungicidal concentration of a composition according to claim 1.

10 6. In a method for inhibiting both fungus growth on and corrosion of a metal normally corrodible by contact with vapor and oxygen, the step comprising maintaining in the immediate presence of said metal an atmosphere containing a corrosion inhibiting and fungicidal concentration of a composition according to claim 2.

15 25

## References Cited in the file of this patent

## UNITED STATES PATENTS

2,225,619 Britton et al. Dec. 24, 1940  
30 2,577,219 Wachter et al. Dec. 4, 1951  
2,717,196 Wachter et al. Sept. 6, 1955

## OTHER REFERENCES

35 Foster: "Chem. Activities of Fungi," 1949, Academic Press Inc., N.Y.C., pp. 515 and 491.